

# UNITED STATES PATENT OFFICE.

ALEXANDER SCHWARCMAN, OF BUFFALO, NEW YORK.

## DRIER AND PROCESS OF MAKING THE SAME.

1,291,186.

Specification of Letters Patent. Patented Jan. 14, 1919.

No Drawing. Application filed February 24, 1911, Serial No. 610,498. Renewed October 13, 1917. Serial No. 196,550.

To all whom it may concern:

Be it known that I, ALEXANDER SCHWARCMAN, a citizen of the United States, residing at Buffalo, in the county of Erie and State of New York, have invented certain new and useful Improvements in Driers and Processes of Making the Same, of which the following is a full, clear, and exact specification.

10 This invention relates to and has for an object to provide an improved oil product and an improved method in the art of treating oils.

This invention particularly relates to the incorporation with raw or normal oil of elements for causing the oil to absorb oxygen readily and to dry rapidly.

Heretofore in treating oil for effecting the quick drying the color of the oil has been changed, that is, it has been darkened and the normal density and viscosity of the oil has been changed, the oil becoming more viscous during the process of treatment.

Oil, particularly linseed oil, consists of fatty acids and glycerin. A part, or all, of the glycerin can be replaced by metals and the resulting products are glycerin on one side and the combination of the respective metals and fatty acids on the other side. The metals of importance in this regard are manganese and lead, as compound of these two metals when introduced into raw linseed oil make it dry much quicker than it would without the presence of these metals. For instance, raw linseed oil under normal conditions will dry in from three to four days. If this oil has added to it, however, compounds of lead or manganese, or a mixture of these metals, the oil will dry in from three to fifteen hours under similar conditions.

The metals above referred to act as catalysts, by which term it is meant that the substance in question does not take a direct part in the chemical reaction but simply assists it.

When linseed oil is exposed to the air it will absorb about sixteen per-cent. of oxygen. This will happen in the raw linseed oil whether the metals above mentioned are present or not. In the presence of compounds of lead or manganese or a mixture of both, the same amount of oxygen will be absorbed but in a very much shorter

time, since the above mentioned metals absorb the oxygen first, then transfer it to the oil thereby expediting the process of absorption of oxygen and the consequent drying of the oil.

In the method which has been largely practised for producing so called boiled oil about two barrels of raw linseed oil are heated in a kettle to about 400 to 500 degrees F., and compounds of lead or manganese are added. The oil is then heated for about five or six hours. The bulk of the lead and manganese are combined with the fatty acids. A small quantity only of such drier can be produced at one operation.

70 The high temperature imparted to the oil has a tendency not only to thicken the oil but to discolor the same. The product is further darkened by the destruction of the part of the glycerin which is replaced by the lead and manganese. This product contains in comparison with that contemplated by the present invention a very diluted drier. To produce "boiled oil" with the drier just described ten per-cent. of the 75 drier will be added to the raw oil which will then be heated to about 250 degrees F. This boiled oil will, of course, have all the shortcomings of the drier incorporated therein. As for instance, it will be 80 darkened, and as the ten per-cent. of drier is very thick in body, on account of the oil having been heated at a high temperature for a number of hours, the resulting product will be more viscous than is raw oil.

85 By my invention however, the desired quantity of some suitable metal base, preferably manganese or lead, or a mixture of these will be incorporated into oil which maintains substantially the characteristics 90 of normal raw oil with the exception that it is given the property of rapid drying.

One method of practising the present improvement is as follows: After the oil has been split into free fatty acids and glycerin 100 by some suitable process, as for instance the Twitchell process, the fatty acids while heated to a temperature below the boiling point of said fatty acids, a practicable temperature to employ being about 240 degrees 105 F., will have added to them chlorid of manganese dissolved in water or a solution of sugar of lead in water. Enough caustic lye is then added to the solution to precipitate the chlorid of manganese as hydrate of man-

60

65

70

75

80

85

90

95

100

105

110

ganese which will dissolve in hot fatty acids while yielding a combination of manganese and the fatty acids, or in the second case hydrate of lead which again combines with 5 the fatty acids yielding a lead combination.

The two metals above referred to may be used together. The lead and manganese may be precipitated in the same manner yielding a lead-manganese combination.

10 When a plurality of metals are used the relative proportions may be varied as occasion demands.

It is of course within the purview of my invention to introduce enough of the metal 15 to completely saturate the fatty acids and obtain a neutral combination. If however, it should be found advantageous to saturate only a part of the fatty acids the resulting combination will consist partially of free 20 fatty acids and partially of a combination of the latter with the above metals.

The fatty acids split from the raw linseed oil easily combine with metallic hydrates which are precipitated in the heated fatty 25 acids and caused to combine therewith preferably while being agitated at a temperature of about 220 degrees F.

By this process large quantities of the 30 drier can be produced at a single operation, and as a low temperature is maintained the metals will combine with the fatty acids without effecting a change in the product. The drier thus obtained is a very highly concentrated one which when added to raw oil, 35 a mixture of raw oil and about two per-cent. of the drier, will produce commercial boiled oil without impairing the color or viscosity of the original raw oil.

To effect the desired drying quality in the 40 so called boiled oil it is necessary merely to incorporate therewith about three-tenths of one per-cent. of the metallic element and by the present method it may be incorporated with the oil and the resulting "boiled oil" 45 will retain the characteristics of pure raw linseed oil with this difference that it will dry in the desired time.

Having thus described my invention, what 50 I claim and desire to secure by Letters Patent is:

1. The improvement in the art of making driers, which consists in adding to free fatty acids at a temperature of about 240 degrees

F. a metallic compound in water, and then adding an alkali, whereby a combination of 55 the metal with the fatty acids in liquid form is produced.

2. The improvement in the art of making driers, which consists in adding to free fatty acids at a temperature of about 240 degrees 60 F. a mixture of chlorid of manganese, sugar of lead and water, and adding an alkali, whereby a lead-manganese combination with a part of the fatty acids, dissolved in the excess of the fatty acids, is produced. 65

3. The art of making driers which consists in incorporating a metal base with an excess of fatty acids at a temperature sufficiently below the boiling point of the said fatty acids to prevent discoloration of the 70 product.

4. The improvement in the art of making driers which consists in adding a soluble metallic salt to an excess of free fatty acids at a temperature below the boiling point of 75 the fatty acids, and then adding an alkali.

5. The improved product which consists of a combination of free fatty acids and a metal base combined in the presence of an excess of the fatty acids and at a temperature below the boiling point of the fatty acids, the product being in the form of a liquid. 80

6. The method of making driers which consists in heating free fatty acids to a temperature below the boiling point thereof, adding to said acids less than their chemical equivalent of a metallic salt in solution and then adding caustic alkali. 85

7. The method of making driers which 90 consists in adding to free fatty acids obtained from linseed oil less than their chemical equivalents of soluble metallic salts and then adding caustic alkali.

8. A light colored liquid drier consisting 95 of a metal combined with the free fatty acids derived from linseed oil, dissolved in an excess of such free fatty acids.

In witness whereof I have hereunto set my hand in the presence of two subscribing witnesses. 100

ALEXANDER SCHWARCMAN.

Witnesses:

GEORGE R. WILKINS,  
W. R. MELVILLE.